

Sept. 16, 1952

H. W. GREIDER ET AL

2,610,928

MINERALIZED BITUMINOUS ROOFING

Filed Aug. 7, 1943

5 Sheets-Sheet 1



INVENTORS  
Harold W. Greider.  
George Arthur Fasold  
BY

Kenny & Kenny  
ATTORNEYS

Sept. 16, 1952

H. W. GREIDER ET AL

2,610,928

MINERALIZED BITUMINOUS ROOFING

Filed Aug. 7, 1943

5 Sheets-Sheet 2



INVENTORS  
Harold W. Greider,  
George Arthur Fosola,  
BY  
Houyoux-Houyoux  
ATTORNEYS

Sept. 16, 1952

H. W. GREIDER ET AL

2,610,928

MINERALIZED BITUMINOUS ROOFING

Filed Aug. 7, 1943

5 Sheets-Sheet 3



Sept. 16, 1952

H. W. GREIDER ET AL

2,610,928

MINERALIZED BITUMINOUS ROOFING

Filed Aug. 7, 1943

5 Sheets-Sheet 4



INVENTORS

Harold W. Greider,  
George Arthur Fasold.

BY

Kenyon-Kenyon

ATTORNEYS

Sept. 16, 1952

H. W. GREIDER ET AL

2,610,928

MINERALIZED BITUMINOUS ROOFING

Filed Aug. 7, 1943

5 Sheets-Sheet 5



## UNITED STATES PATENT OFFICE

2,610,928

## MINERALIZED BITUMINOUS ROOFING

Harold W. Greider, Wyoming, and George Arthur Fasold, Mount Healthy, Ohio, assignors to The Philip Carey Manufacturing Company, a corporation of Ohio

Application August 7, 1943, Serial No. 497,809

2 Claims. (Cl. 117—168)

1

This invention relates to roofing. It relates particularly to roofing embodying bituminous material as waterproofing.

Heretofore bituminous prepared roofing has been very extensively manufactured using as a base a fibrous web such as roofing felt, impregnating the fibrous web with a bituminous material, and coating the impregnated web with a weather-resistant bituminous coating composition. The bituminous coating composition usually contains a mineral filler such as slate flour or powdered limestone in amounts less than about 40% by weight of the bituminous coating composition. Usually there is applied to the bituminous coating on the surface intended to be exposed to the weather a suitable granular material such as slate granules or more finely divided mineral surfacing material such as talc or mica. Finely divided materials such as mica flakes, talc, silica dust or the like may be made adherent to the non-weather exposed surface of the roofing to prevent sticking of adjacent layers of the roofing material in the package.

The term "roofing" is used herein in the broad sense as referring to water- and weather-resistant coverings such as shingles (individual or strip shingles), roofing tiles, cap sheets, sidings, roof deck coverings made from such preformed materials, built-up roofings, and the like.

The bituminous roofings of the character aforesaid that have been manufactured and sold heretofore have relatively low fire-resistance. The most widely-accepted tests for determining the fire-resistant properties of roofing are those prescribed by Underwriters' Laboratories, Inc., of Chicago, Illinois. According to the tests prescribed by Underwriters' Laboratories, Inc., fire retardant roofings are placed in three classifications, depending upon their ability to pass the tests required for each classification, these classifications being Class A, Class B and Class C. The Class C rating is the lowest fire-retardant rating and serves to distinguish roofings having appreciable fire-retardant properties from roofings having little or no fire-retardant properties such as untreated wood shingles which, of course, are readily ignited and tend to burn freely. So far as we are aware, prepared bituminous roofings of the type heretofore on the market made on an organic fiber felt base have not been able to attain, regardless of the thickness thereof or the number of thicknesses, a rating of Underwriters' Laboratories, Inc. higher than a Class C rating. The Class A rating is the highest rating awarded by Underwriters' Laboratories, Inc. and is reserved for such highly fire-retardant roofings as asbestos-cement shingles of the double-coverage

2

type. Class B is an intermediate rating and is, for example, awarded to roofings such as single-coverage asbestos-cement shingles. A brief description of the Class A, Class B and Class C fire-retardant tests of Underwriters' Laboratories is contained in our pending applications for Roofing, Ser. No. 370,636, filed December 18, 1940 (Patent No. 2,326,723) and Ser. No. 399,024, filed June 20, 1941 (Patent No. 2,326,724).

It is a purpose of this invention to improve the fire resistance of roofings comprising a layer of thermoplastic material such as bituminous material. Thus, for example, we have found that a roofing material which comprises an organic fiber felt base and a bituminous waterproofing coating can be made according to this invention, at the cost of ordinary bituminous roofing material, that is so highly fire-retardant that a three-layer covering on a combustible roof deck will satisfactorily withstand exposure to the Class A fire-retardant tests prescribed by Underwriters' Laboratories, Inc. We have found further that such roofing material embodying our invention, when applied so as to provide two layers, will satisfactorily pass the Class B fire-retardant tests prescribed by Underwriters' Laboratories, Inc.

The importance of fire-resistant properties for roofing is self-evident. Certain roofings such as asbestos-cement shingles, tile and the like have high fire resistance but such roofings are very costly as compared with asphalt felt roofings, and for this reason asphalt-felt roofings are very extensively used on all kinds of structures notwithstanding the limited fire-protection that is afforded by this type of roofing. According to this invention, asphalt-felt roofings can be made without substantial increase in cost which are comparable in fire-retardant properties to relatively much more costly roofing constructions such as asbestos-cement, tile and the like.

Substantially all bituminous roofings comprise a strain-resisting base or foundation sheet such as roofing felt which is coated with a bituminous coating that provides waterproofing and weather resistance. This invention has to do with the coating material rather than the base sheet. While the base sheet might be made of non-combustible material, the non-combustibility of the base sheet does not solve the problem if the bituminous coating itself burns or tends to flow so as to spread the flame. According to the present invention, the waterproofing coating is rendered highly fire-resistant so that, even when applied to a base sheet of combustible organic fibers, roofing can be made which has the high degree of fire resistance mentioned above.

In our aforesaid copending application, Ser. No.

370,636 (Patent No. 2,326,723), we have described and claimed bituminous roofing comprising a bituminous waterproofing composition that, while highly fire resistant, possesses physical properties such as pliability and resistance to flexure that correspond in a general way with bituminous roofings of similar character previously manufactured and sold. The bituminous coating composition of the roofing disclosed and claimed in our application Ser. No. 370,636 contains bitumen having a softening point above 160° F. and of the range 45% to 70% by weight of the coating composition. The coating composition also contains filler material of the range 30% to 55% by weight of the coating composition and in the form of finely divided solid water-insoluble heat-resistant mineral material of special character that is described, illustrated and defined in our application Ser. No. 370,636.

The present invention has to do with roofing comprising more highly mineralized bituminous waterproofing coatings than those described and claimed in our aforesaid application Ser. No. 370,636, namely, coating compositions containing more than 55% by weight of finely divided solid water-insoluble heat-resistant mineral filler. Such roofings at ordinary temperatures are somewhat stiffer and less pliable than the roofing disclosed in our application Ser. No. 370,636 and are especially suitable for certain types of roofing where toughness and resistance to flexure are desirable and a high degree of pliability is not essential. For example, the roofing of the present invention is desirable as a weather- and fire-resistant surface layer of built-up roofing. Ordinary built-up roofing, especially when laid over fibrous or cellular heat insulation material, is indented quite readily and is subject to injury due to people walking thereon. The roofing of the present invention is suitable for improving the fire resistance and resistance to indentation and rupture of built-up roofing since the roofing of the present invention not only has very high fire resistance but also has considerably more toughness and resistance to flexure than ordinary roofing materials. For use as the upper layer of built-up roofing, roofing material embodying this invention may be made up into sheets or may be made in the form of tile-like pieces adapted to be bonded in place by a bituminous adhesive.

The fire-resistant bituminous composition of the present invention may likewise be used in the manufacture of multi-ply prepared sheets consisting of a plurality of layers of bituminized mineral fiber or organic fiber felt or other fabric having one or more layers of bituminous composition therebetween. This type of roofing is inherently semi-rigid in character and the highly mineralized fire-resistant bituminous composition of this invention is well suited for use as a weather- and waterproofing layer therein either between the plies of fabric or as a surface or backing layer or both. One type of roofing made in this way has an unsaturated sheet of asbestos felt as the top layer so as to provide resistance to fire caused by falling sparks such as are likely to occur in the vicinity of railroads, smelters, etc. According to the present invention, greater weather-resistance and at the same time greater fire-resistance is obtainable by providing as the upper or weather-exposed surface of this type of prepared roofing a bituminous surface layer consisting of the highly mineralized fire-resistant bituminous composition of this invention.

While the roofing of this invention is particularly suited for purposes such as those above

mentioned, roofing in the form of shingles, siding and the like may embody the highly fire-resistant bituminous coating composition of this invention. When shingles, either individual or strip shingles, are prepared according to this invention, they usually are somewhat more stiff than conventional bituminous prepared roofing materials, but they are well suited for use wherever bituminous shingles and the like may be used, and are thus of special advantage in regions where high winds are likely to be encountered, as, due to their stiffness, they resist blowing up or "fluttering" in the wind. The roofings of the present invention usually have higher tensile strength than conventional roofings and this feature also is advantageous for certain purposes.

In our application Ser. No. 497,805 which was filed simultaneously with our present application and which has resulted in Patent No. 2,424,234, we have described and claimed a bituminous composition especially adapted for use as the mopping asphalt in the construction of built-up roofings, the composition possessing high fire-resistance by virtue of its formulation so as to comprise bitumen having a softening point between about 80° F. and about 200° F. and of the range 35% to 60% of the composition, so as to comprise intimately commingled and distributed uniformly throughout the bitumen finely-divided solid water-insoluble heat-resistant mineral filler which is of the range 40% to 65% by weight of the composition with at least 2/3 by weight thereof passing a 100 mesh testing sieve, and so as to have a Wagner-Bowen plasticity value at 400° F. not substantially greater than 250 grams, the filler in the composition having a flow resistance coefficient of at least 75 when the composition is subjected to the flow resistance test that is defined in the application. The bituminous composition disclosed in our aforesaid application Ser. No. 497,805 successfully solved the specific problem of providing a mopping asphalt suitable as the waterproofing adhesive between the plies of built-up roofing which is capable of application on the job using an implement such as a mop and which at the same time overcomes the low order of fire resistance that is an inherent attribute of conventional mopping asphalt compositions.

As distinguished from the mopping asphalt adhesive composition disclosed in our aforesaid application Ser. No. 497,805, the invention of our present application is directed to the provision of highly mineralized roofing products of very high fire resistance which comprise a base sheet and coating layer and which have the properties, advantages, and fields of use that have been indicated hereinabove. The requirements for affording a highly fire resistive roofing product according to our present invention differ markedly from the requirements for affording a highly fire resistive mopping asphalt composition according to the invention disclosed in our said application Ser. No. 497,805 in several significant respects one of which is that while the mopping asphalt composition disclosed in our said application is limited to one wherein the Wagner-Bowen plasticity value at 400° F. is not substantially greater than 250 grams, the highly mineralized coating composition combined with a base sheet according to our present invention comprehends coating compositions whose Wagner-Bowen plasticity value at 400° F. is substantially greater than 250 grams while not being substantially greater than 1500 grams. Moreover, the coating of the roofing product of our present invention comprehends

coatings having the commercially important advantage of being highly blister resistant, the coatings in such case utilizing bitumen having a softening point above 200° F. These and other distinctions will be apparent from the following description of our invention.

In the preparation of bituminous waterproofing coatings for bituminous roofing, the incorporation in the bituminous waterproofing coating composition of mineral filler material such as powdered limestone or slate flour has little effect upon the fire resistance of the roofing when this filler is used in amounts such as the amounts previously employed in the manufacture of bituminous roofings, usually about 30% to 40% by weight of the bituminous composition. Such bituminous compositions when used as the waterproofing layer overlying a base sheet of felted fiber or the like tend to be consumed when subjected to flame and to flow down an inclined roof deck leaving the underlying fibrous sheet exposed to the destructive action of the heat of the flame. Thus a filler material such as powdered limestone or slate flour, even when incorporated in a bituminous composition to an extent as high as 55% by weight of the bituminous coating composition, has little effect in reducing the combustibility and resistance to flowing of the bituminous coating composition.

We have found that in the formulation of bituminous coating compositions suitable for roofing there is a critical point below which a finely-divided mineral filler exerts little, if any, effect upon the combustibility and flow resistance of bituminous coating compositions but above which even slight further additions of the mineral filler exert a profound effect upon the combustibility and flow resistance of the bituminous coating composition. This critical point usually is in the neighborhood of the maximum amount of the filler in question that can be successfully mixed and spread as a satisfactory coating upon a base sheet such as a sheet of asphalt-saturated organic fiber felt. This critical point is different for different mineral fillers and usually is found to occur at a mineral filler content of about 60% to about 80% by weight of the bituminous composition, depending on the particular mineral filler used. The critical point also is affected by the type of bitumen that is used as the waterproofing base for the bituminous composition.

When reference is made herein to "bitumen," this term is used herein in reference to asphalt, pitch, tar and the like, by itself and unmixed with filler. When, on the other hand, reference is made herein to a bituminous material, or a bituminous composition, or a bituminous coating, or a bituminous layer, reference is made to a material, composition, coating or layer comprising bitumen either with or without a filler.

It is a feature of this invention that there is employed as bituminous coating composition of roofing material, highly mineralized bituminous composition within the narrow zone above the critical point at which the coating composition becomes highly resistant to flow when exposed to flame temperature and below the point at which the coating becomes of excessively high plasticity or consistency at 400° F. When the bituminous coating is formulated so that its properties be within this zone, we have found that a satisfactory roofing of high resistance to fire is obtained. When a roofing carrying a bituminous composition is formulated within the limits just mentioned, we have found that the

composition upon being exposed to temperatures at or approaching flame temperatures, instead of burning and flowing, remains in place due to the filler constituting a skeletal mat that remains stable and coherent and that holds the bitumen in place so that it does not flow down an inclined roof deck, e. g., a roof deck having a 30 degree inclination to the horizontal, leaving the underlying material such as a combustible organic felt base sheet exposed to the flame. Another attribute of the roofing is that the fire-resistant bituminous coating when exposed to high temperatures at or approaching flame temperatures tends to result in a coherent mat-like mass which has high heat insulating properties and in preferred embodiments develops pores therein and which effectively shields an underlying combustible roof deck from the heat of the flame. Another attribute of the fire-resistant coating is that it is highly resistant to combustion so that, if it tends to char upon exposure to flame, the charring and combustion are very gradual and discontinue without substantial spreading as soon as exposure to flame is discontinued. By formulation of the bituminous coating composition within the limits specified herein and in the claims, these effects whereby the filler retains the bitumen even when the coating is heated to a temperature at or adjacent flame temperature and whereby the bitumen upon exposure to flame carbonizes as a cementitious charred mass that forms with the skeletal mat of fiber a coherent fire-resistant heat insulating protective layer, are attained, and if these critical limits are departed from the roofing no longer has the fire resistance of the roofing herein defined but fails in fire resistance for such reasons as excessive combustibility of the coating, bleeding and running of the bitumen, flowing of the coating as a whole so as to expose the underlying base sheet, excessive separation from the base sheet, disintegration or excessive cracking of the coating on exposure to flame, and the like.

Other features of this invention relate to the disposition of the special coating material in strata in roof deck coverings.

In the case of mineral filler materials such as slate flour or powdered limestone that are non-fibrous, the critical point at which the pronounced flow resistance of bituminous compositions when exposed to flame temperature is attained, is usually in the upper portion of the filler range mentioned above. The critical point in the case of such non-fibrous mineral filler materials can be modified so that the critical change will occur with a lesser total filler content by mixing with the powdered non-fibrous filler a finely-divided mineral fiber filler passing a 6 mesh testing sieve and retained on a 200 mesh testing sieve. Fibrous mineral filler is more effective in affording high flow resistance than is a non-fibrous mineral filler, although, as will be pointed out more in detail hereinbelow, certain screen gradings of fibrous mineral filler are considerably more effective than others. It is preferable, therefore, to employ in the practice of this invention a special bituminous composition comprising fibrous mineral of such screen fractions and in such amounts relative to the bitumen in the composition as to impart very high flow resistance and fire-resistant properties to the roofing.

In order to afford a better understanding of this invention, it will be described for purposes of exemplification in connection with a typical em-

bodiment. The roofing material of this embodiment is composed of strain-resisting roofing felt, a top weather surface coating of special bituminous coating composition, a surface layer of mineral granules partially embedded in the surface coating, a thinner layer of the special coating composition on the back of the felt base sheet, and finely-divided dusting material adherent to the back layer of the special bituminous coating composition.

In the exemplary embodiment, the base or foundation sheet is ordinary roofing felt made of vegetable and animal fibers, e. g., a roofing felt made from organic fiber stock weighing about 6 pounds per 100 square feet. The felt is impregnated with a suitable impregnating material, e. g., a conventional bituminous roofing saturant having a softening point of about 120° F. to about 170° F. The base sheet as thus composed has little fire resistance and, when exposed to fire, is consumed quite readily.

A typical example of the special coating composition may be made as follows: The bitumen used in the coating is preferably a residual asphalt flux from the refining of Mid-Continent petroleum which has been oxidized as by air blowing until it has a softening point of about 200° to 210° F. and constitutes about 32% by weight of the composition. With this asphalt there is intimately commingled and distributed uniformly throughout finely-divided mineral filler which constitutes 68% by weight of the composition. The filler consists of powdered limestone which constitutes about 47% by weight of the composition and asbestos dust which constitutes about 21% by weight of the composition. The powdered limestone is limestone which has been reduced to a pulverulent condition, about 85% by weight of it passing a 200 mesh testing sieve. The asbestos dust is such that nearly all passes a 14 mesh testing sieve, with about 75% by weight retained on a 200 mesh testing sieve and about 25% by weight passing a 200 mesh testing sieve. Such asbestos dust is considerably finer in particle size than the asbestos which is ordinarily placed on the market and which is known in the art as fiber. Heretofore such asbestos dust has generally been discarded in enormous amounts in dumps at the mines as a waste product while the usual asbestos fibers of commerce have been recovered and sold.

The screen grading of the asbestos dust used in the coating composition of the example of this invention appears below. The percentages given are percentages by weight contained in the bituminous compositions. A given screen grading such as that passing a 6 mesh testing sieve and retained on an 8 mesh testing sieve is indicated as (-6+8). Other screen gradings are indicated similarly.

| Screen gradings                    | Percent contained in bituminous composition |
|------------------------------------|---------------------------------------------|
| -6+8                               | .1                                          |
| -8+10                              | .2                                          |
| -10+14                             | .3                                          |
| -14+20                             | .3                                          |
| -20+28                             | .4                                          |
| -28+35                             | 1.5                                         |
| -35+48                             | 3.0                                         |
| -48+65                             | 2.5                                         |
| -65+100                            | 2.5                                         |
| -100+150                           | 2.5                                         |
| -150+200                           | 2.0                                         |
| -200                               | 5.7                                         |
| Total asbestos dust in composition | 21.0                                        |

In preparing the special coating material, the asphalt is heated to a heat-liquefied condition and the asbestos dust and limestone dust are thoroughly mixed therewith. The mixing preferably is carried out at a temperature of about 375° F. to 475° F. It is important that the bitumen and finely-divided filler be thoroughly mixed and intimately commingled so that the composition of the coating with respect to the distribution of the filler therein is uniform throughout. The composition should be applied to the felt base sheet while in a thoroughly mixed condition so that the resulting layer is substantially uniform in consistency and in thickness. In the typical embodiment herein described, the coating is applied to the felt base sheet at the rate of about 45 pounds per 100 square feet. Before the coating cools to atmospheric temperature, a conventional surfacing material such as slate granules, can be applied to the surface for weather exposure and these granules are partially embedded in the coating composition. The granular surfacing material is preferably non-combustible and, while employed, is not relied upon to impart fire resistance to the roofing. On the opposite side of the roofing material, there may be applied a thin coating of bituminous coating material, e. g., an asphalt having a softening point of about 200° to 240° F., so as to weigh about 5 pounds per 100 square feet, and finely-divided dusting or anti-stick material such as talc or mica dust or similar material may be applied and partially embedded in the back coating. Preferably, for maximum fire resistance, the back coating should be special coating composition embodying our invention.

The roofing thus prepared may be packaged in sheet form, or, alternatively, may be cut into sections suitable for shingles or tile-like units. The roofing weighs about 95 pounds per 100 square feet. Of this weight, about 30% by weight is in the form of mineral granules adherent to one side and finely-divided, dusting material adhered to the other side, the balance of the roofing being the felt, the bituminous impregnating material and the bituminous coating material.

The special bituminous coating composition may advantageously be mixed and applied in the manner mentioned in our said application Ser. No. 370,636 (Patent No. 2,326,723). As stated in said application, the coating composition may, if desired in order to increase the resistance of the applied coating to blistering, be applied using the method and apparatus of our Patents Nos. 2,105,531 and 2,159,587, but this is not essential.

The roofing material above described can be made up into suitable preferred roofing materials and into suitable roofing structures, description of typical roofing structures being facilitated by reference to the accompanying drawings, wherein

Fig. 1 is a plan view of prepared roofing material embodying our invention in the form of a rectangular unit;

Fig. 2 is a fragmentary sectional view on an enlarged scale of the roofing material shown in Fig. 1;

Fig. 3 is a plan view, somewhat diagrammatic, of a built-up roofing embodying roofing made according to our invention;

Fig. 4 is a fragmentary cross-sectional view on an enlarged scale of the built-up roofing shown in Fig. 3;

Fig. 5 is a plan view of prepared roofing material embodying our invention that has been cut in a form suitable for use as a strip shingle;

Fig. 6 is a fragmentary sectional view on an enlarged scale of the roofing material shown in Fig. 5;

Fig. 7 is a sectional view of a roof covering composed of strip shingles laid on an inclined roof deck without showing the component layers of the individual shingles;

Fig. 8 is an enlarged sectional elevational view of a portion of the roof shown in Fig. 7;

Fig. 9 is similar to Fig. 8 except that the roofing is shown as it appears after exposure to flame temperature;

Fig. 10 is a fragmentary sectional view of another embodiment of this invention;

Fig. 11 is a side elevation partly in section of a testing device for testing the flow resistance of filler material as incorporated in a bituminous composition;

Fig. 12 is a plan view partly in section of the testing device;

Fig. 13 is a front elevation of the test panel assembly;

Fig. 14 is a side elevation of the test panel assembly;

Fig. 15 is a plan view of the test panel assembly with parts thereof broken away;

Fig. 16 is a perspective view of the frame and guard plate used in the test panel assembly;

Fig. 17 is a longitudinal sectional detail view on an enlarged scale of the orifice in the gas line leading to the burner of the testing device;

Fig. 18 is an end elevation of the Wagner-Bowen plasticimeter testing device;

Fig. 19 is a plan view of the plasticimeter;

Fig. 20 is a front elevation partly in section of the plasticimeter;

Fig. 21 is a side detail elevation of the drag tool and drag tool support of the plasticimeter;

Fig. 22A, Fig. 22B, and Fig. 22C are views of the smoothing blade of the plasticimeter taken respectively in elevation normal to the line A—A of Fig. 19, from the bottom, and in elevation from the back in the direction of the line A—A of Fig. 19;

Fig. 23A, Fig. 23B, and Fig. 23C are views of the mixing blade of the plasticimeter taken respectively in elevation normal to the line B—B of Fig. 19, from the bottom, and in elevation from the back in the direction of the line B—B of Fig. 19.

Prepared roofing material embodying this invention may be in the form of a unit 30 which may be of rectangular shape as shown in Fig. 1 or of any other desired shape. The cross section of this embodiment is shown in Fig. 2 and comprises a base or foundation sheet 31 of bitumen impregnated roofing felt. Overlying the roofing felt is the coating 32 of special coating composition having adherent to the surface thereof and partially embedded therein slate granules 33. While the prepared roofing material is illustrated in the form of a unit of special shape, the roofing material may, of course, be in the form of larger sheets or in the form of rolls of indefinite length of the roofing material.

In Figs. 3 and 4, roofing embodying the special coating composition of this invention is shown in connection with built-up roofing. The roof deck 34, has sheets 35 of red rosin paper or the like applied thereto as a single thickness. Overlying the red rosin paper are two layers 36 and 37, the layer 36 consisting of bituminized felt 36a and bituminous coating 36b and the layer 37 consisting of bituminized felt 37a and bituminous coating 37b. The layers 36 and 37 are bonded

together by a layer 38 of mopping asphalt. Adherent to the upper side of layer 37 by a layer of mopping asphalt 39 are a plurality of the tile-like roofing elements 30 which comprise the layer of bituminized felt 31, the layer of special bituminous coating composition 32 and surfacing granules 33. In such a built-up roofing the tile-like roofing elements 30 provide a highly fire-resistant surface coating. Moreover, since these roofing elements carry a highly mineralized surface coating, they have more rigidity and strength than ordinary roofing materials used for the surface of built-up roofings and provide a surface that will withstand considerable walking upon and the action of other loads that tend to indent or rupture the surface of the roof covering.

By causing the layers 36b and 37b of the bituminous composition to be of the special character described herein or to be of the special character described in our application Ser. No. 370,636 above mentioned, the built-up roofing as a whole can be made so as to have extremely high resistance to fire.

In Fig. 5 prepared roofing embodying the special coating composition of this invention is shown as cut in the form of a strip shingle 40. In cross-section the prepared roofing appears as in Fig. 6 and comprises a base or foundation sheet 41 with an overlying layer 42 of the special bituminous coating composition. Granules 43 are partially embedded in the layer 42. Adherent to the back of the roofing material is a layer 44 of the special bituminous coating material in which is partially embedded dusting material 45.

In Fig. 7 is shown a typical roofing structure in place on a roof deck comprising boards 46 which serve as a support for the shingles 40. The shingles 40 may be 16 inches from the butt to the top and may be laid with a 5-inch exposure, thereby affording triple coverage over all parts of the roof deck except for the double coverage area beneath the cutouts. The component parts of the individual shingles appear in detail on the enlarged fragmentary view shown in Fig. 8.

A roofing structure of the character described in the above example has extremely high fire-resistance. Thus a roofing such as that shown in Figs. 7 and 8 comprising three thicknesses of the special roofing of this invention will withstand the Class A fire-retardant tests as prescribed by Underwriters' Laboratories, Inc., in their published instructions. As mentioned above, we do not know of any commercial prepared bituminous roofing made on a felt base of organic fibers which, irrespective of the weight of the roofing material or the number of layers or plies that are applied to the roof deck, will successfully pass either the Class A fire-retardant tests or will even pass the Class B fire-retardant tests of Underwriters' Laboratories, Inc.

When ordinary bituminous prepared roofing such as ordinary asphalt shingles is subjected to the Class A burning brand test, the bituminous coating composition when exposed to the burning brand melts and as a mass starts running down the surface of the roof. The melted asphalt also starts to burn and the burning asphalt in running down the roof spreads the fire. The coating composition that runs down the roof leaves the bituminous organic fiber felt base exposed, which, being readily combustible, starts burning so that the fire goes through the roofing

quite readily and ignites the combustible roof deck in a relatively short time.

By way of contrast, our improved roofing made as above described by way of example behaves very differently when subjected to the same burning brand test. The behavior of the roofing material as applied to a roof deck in three layers, e. g., as shown in Figs. 7 and 8, is indicated roughly in Fig. 9. During exposure to the flame, the bitumen and filler remain in place and the filler provides a skeletal mat so that, as the bitumen in the coating carbonizes, a coherent protective mat-like layer is formed that shields the underlying roof deck from the heat of the flame. Moreover, especially when a mineral filler such as asbestos dust is present that contains water of constitution liberatable at or adjacent flame temperature, small bubbles 47 form in the residual coherent mat-like mass that tend to augment the heat insulation effectiveness of the carbonized residue. In the roof covering structure as a whole as illustrated in Fig. 9, the upper layer of special coating composition has become expanded and has become somewhat irregular but still remains as a protective coherent heat-insulating mat-like mass. The layer of felt 41 may be carbonized and to a considerable degree may have disappeared, leaving air pockets 48 with some residual carbonized material. The intermediate layer of special coating material is also expanded and remains in place as a protective mat. The intermediate layer of felt is charred but is better preserved than the uppermost layer of felt. The bottom layer of special coating composition is less severely carbonized than the upper layer and is likewise substantially expanded. The bottom layer of felt is fairly well preserved and the underlying board, if charred at all, has not become ignited. It usually takes the burning brand used in making the Underwriters' Class A burning brand test about 30 to 45 minutes to burn out. During this time, the upper surface of the uppermost layer 42 may become red-hot, but the heat insulating effect of the underlying carbonized residue of layers 42 (and to a lesser degree of the thinner layers 44) is so great that the board 46 does not become ignited and in some cases does not even appear scorched. During this test, the effect of the flame on the roofing is confined to the area beneath and closely adjacent to the position of the burning brand, and, when the brand burns out, all charring of the roofing soon ceases and the roofing cools down. The behavior of the roofing hereinabove described under the Class A flame exposure test is generally similar to that just described in connection with the Class A burning brand test. Such roofing also passes the Class A flame spread test. In the case of built-up roofing such as that shown in Figs. 3 and 4, the behavior upon exposure to flame, if the layers of coating composition are of the special character herein defined, will be similar to that just described. If roofing is made up so as to provide double coverage instead of triple coverage, roofing of the composition aforesaid will pass the Class B fire-retardant tests of Underwriters' Laboratories, Inc. Instead of using strip shingles, the roofing shown in Figs. 7, 8 and 9 may, if desired, be made up with individual shingles embodying the special coating composition of this invention.

The fire-resistance of the bituminous coating composition described in the foregoing exemplary embodiment of this invention is obtainable due to the fact that the filler-asphalt mixture is

formulated within the critical zone or range determined on the one hand by the minimum flow resistance coefficient under the flow resistance test at flame temperature to be described below, and, on the other hand, by the maximum plasticity value at 400° F. under the plasticity test which also will be described below. As aforesaid, a filler material such as the filler material used in the foregoing exemplary embodiment of this invention exercises only very slight effect on the fire-resistance of roofing, which effect is negligible as far as useful increase in fire-resistance is concerned, even when the filler material is used in considerable quantities up to about 55% by weight of the composition. Thus utilizing the filler of the foregoing example which consists substantially of 1 part of asbestos dust for each 2 1/4 parts of powdered limestone, the flow resistance coefficient of the filler is only about 50, even when the filler constitutes about 45 by weight of the composition, the balance of the composition consisting of asphalt having a softening point of 205° F. This is somewhat higher than the flow resistance coefficient of 22 which is obtained when the same asphalt is used but without any filler being included therein but still represents a very low and inadequate degree of flow resistance. However, by further addition of the filler material, other conditions of the test and of the tested sample remaining the same, the flow resistance coefficient of the filler increases very rapidly and, in the case of the exemplary embodiment hereinabove described, becomes increased to the maximum possible value of 100, namely, a condition such that there is no flow whatever of the bituminous coating composition when exposed to flame temperature. It is apparent, therefore, that there is critical and sharp change that occurs and brings about a greatly modified physical condition of the bituminous composition and at which the action of the filler changes from affording only a low flow resistance coefficient to affording a very high flow resistance coefficient. When the condition of high flow resistance coefficient is attained, there is a cooperative action between the filler and the bitumen in the coating. On the one hand, the filler material serves to prevent the bitumen under the heat of the flame from running and burning. On the other hand, the bitumen during carbonization as held in place by the filler provides a carbonaceous binder that cements the filler material together as a coherent mass that has substantial inherent strength and that prevents the filler from crumbling and being displaced. The result is a mat-like mass of considerable body and coherence that has very high heat insulating effectiveness and that serves as a very effective barrier in protecting the underlying roof deck from the heat of the flame.

We have found that the flow resistance coefficient of a filler or filler mixture as dispersed in the bitumen of a bituminous composition is a definite and measurable property that, while a different type phenomenon, may be likened to the property of certain substances of raising or lowering the boiling point of a liquid in which the substance is dissolved. We have also found that high fire-resistance is provided if the flow-resistance coefficient is sufficiently high. In order to accurately determine the flow-resistance coefficient and thereby enable us to precisely define the highly fire-resistant roofings of this invention, we have devised a test whereby the flow-resistance

coefficient of a particular filler or filler mixture in a bituminous composition under conditions of exposure to fire may be measured. The test consists in directing a flame against an inclined specimen of roofing that carries a coating consisting of the bitumen and the filler or filler mixture to be tested, under precisely-controlled conditions determined by the construction and operation of the testing apparatus. The following is a description of the controlled conditions of the test, reference being made to Figs. 11 to 17 of the drawings.

Samples carrying the bituminous composition containing the filler or filler mixture to be tested are made by applying the bituminous coating composition to the base sheet material so that the coating weighs 30 pounds plus or minus 2 pounds per 100 square feet.

The test is made in a wind tunnel 50 having a fan 51 at one end and a stack 52 at the other end. The tunnel is made of  $\frac{1}{4}$  inch thick asbestos-cement lumber and has two windows 53 and 54 therein which can be opened and closed by any suitable means (not shown).

Within the tunnel are the burner and testing deck which are located between two shields 55 and 55<sup>1</sup> of the asbestos-cement lumber spaced  $12\frac{1}{4}$  inches apart, and which are rigidly mounted on the asbestos-cement slab 56. The inclined test deck is indicated generally by the reference character 57 and comprises a lower frame-like member 58 having  $\frac{1}{4}$  inch pegs 59 projecting from the face adjacent the upper and lower margins. Between the pegs 59, strips 60 of asbestos-cement boards  $1\frac{3}{4} \times 12 \times \frac{1}{4}$  inches are placed. One ply 12 x 12 inches of the prepared coated sample 73 to be tested is placed on the asbestos-cement boards 60 followed by an L-shaped guard plate 61 which covers the bottom edge of the sample. The assembly is held down by an iron frame 62 and held in place by thumb screws 63.

After the test deck has been assembled, it is placed on the inclined support 64 which has an opening in the back underneath the strips 60 and which has side flanges 65 to protect each side of the test panel. The support 64 comprises a baffle 66 to prevent the flame licking around behind the test deck. The support, which is made of iron, is mounted on the asbestos-cement slab 56 which measures 12 x 40 x 1 inches. The parts for carrying the test deck are also made of iron. An iron bar 67, 12 x 1 x  $\frac{1}{4}$  inches is placed across the top edge of the deck to protect the sample at this point.

In front of the test deck is the burner 68 comprising an iron pipe having an inside diameter of .472 inch and an outside diameter of .675 inch, with 17 holes .078 inch in diameter and  $\frac{1}{2}$  inch apart disposed at an angle that is parallel with the plane of the test deck. The burner is provided with an inlet line 69 controlled by a shut-off valve 70. In the line 69 is an orifice 76,  $\frac{5}{64}$  inch in diameter, that is located in the housing connections 71. Between the valve 70 and the orifice is a manometer 72. By this arrangement, a supply of gas under constant pressure can be obtained, thereby obtaining a steady flame of constant intensity during the test.

At the base of the test deck and between the burner and the deck holder is placed a pan 74,  $\frac{3}{4} \times 1 \times 10$  inches, which collects any bituminous coating material that flows from the sample during the exposure to the flame. This pan is provided with a removable cover 75.

The dimensions of the different parts of the

testing apparatus shown in the drawings as used by us are as follows:

|    | Inches          |    | Inches          |
|----|-----------------|----|-----------------|
| a  | 24              | o  | 8               |
| b  | 38              | p  | 2               |
| b' | 6               | q  | $\frac{3}{4}$   |
| c  | $18\frac{1}{2}$ | r  | 1               |
| d  | 72              | s  | 12              |
| e  | $16\frac{1}{2}$ | t  | 7               |
| f  | 10              | u  | $10\frac{1}{2}$ |
| g  | $12\frac{1}{4}$ | v  | 12              |
| h  | 38              | w  | 12              |
| i  | 64              | x  | 1               |
| j  | 32              | y  | 12              |
| k  | 24              | y' | 1               |
| l  | 24              | z  | 6               |
| m  | 40              | aa | 12              |
| n  | 27              | bb | 1               |

In carrying out the test, the apparatus is first assembled, and the burner is lighted so as to provide a pilot flame that is about  $\frac{1}{2}$  inch in length when the fan is operating. The windows 53 and 54 are then closed and the room in which the apparatus is placed is arranged so that there will be relatively constant conditions during the test. The temperature and relative humidity of the room should be approximately 80° F. and 40%, respectively. The fan should generate a wind velocity of about 150-155 ft. per minute at the portion of the deck exposed to the flame. The valve 70 is then opened until a flame about 8 to 9-inches long is produced having a temperature of about 1325-1370° F. When the valve 70 is opened to produce such flame, a timing device is started. After the sample has been exposed to the flame for a period of five minutes, the flame is turned off and simultaneously the cover 75 is placed over the top of pan 74 so as to prevent any further bituminous composition that may flow down the test deck from collecting in the pan. Before the commencement of the test, the pan 74 is carefully weighed and at the conclusion of the test is again weighed, the difference in weight being the number of grams of bituminous coating material that has flowed into the pan. Before making the test, the weight of the bituminous coating on the test sample is determined by weighing the base sheet material before the bituminous coating is applied thereto and weighing the complete sample, the difference being the weight of the coating.

The coefficient of flow resistance is computed according to following expression.

$$55 \quad \frac{\text{weight in grams of coating collected in pan} \times 100}{100 - \text{total weight in grams of coating prior to test}}$$

For example, if the weight of the bituminous coating on the sample was 1000 grams prior to testing and 50 grams of the coating were collected in the pan during the test, the coefficient of flow resistance would be

$$60 \quad 100 - \frac{50 \times 100}{1000} = 95$$

65 If no coating composition flows into the pan, then the flow resistance coefficient is 100 which is the maximum attainable.

70 The flow resistance coefficient is primarily a function of the filler contained in the bituminous composition since the greatly-increased flow resistance of the coating, if attained, is due to presence of the filler in an amount that equals or exceeds the critical amount for the filler undergoing test. It may be mentioned, however,

that the amount of a given filler that is critical will usually vary somewhat depending upon the bitumen that is used in the bituminous composition. Thus the critical amount of filler for a so-called "cracked asphalt," namely, oxidized asphaltic cracking still residue, is usually somewhat less than for a straight run asphalt residue.

Another factor that influences the flow resistance coefficient somewhat is the character of the surface to which the bituminous coating composition is applied. In the manufacture of roofing material, a typical asphalt saturated organic fiber felt base sheet weighs about 30 lbs. per 100 square feet which is saturated to the extent of about 175% by weight with asphalt having a softening point of about 150° F., so for most purposes an asphalt saturated felt such as this may be used in making the test. However, for bituminous compositions which have incorporated the critical amount of filler to render the composition highly flow-resistant, the asphalt in an asphalt saturated base sheet exerts an effect as a lubricant at the interface between the base sheet and the coating composition which tends, depending upon the amount of asphalt in the base sheet, to lower somewhat the flow resistance coefficient as determined by the test. This effect can be counteracted by indenting or otherwise causing the surface of the felt base sheet to be rougher than normal. By using a dry or unsaturated felt base sheet, especially base sheet material having relatively coarse fibers, the flow resistance coefficient of the bituminous composition per se is attained without being influenced by an effect that the bitumen in the base sheet may have. However, since the special coating composition of this invention may be utilized overlying the surface of different kinds of base sheet material, it is best to carry out the flow resistance test using as the base sheet for the test sample the kind of base sheet that is to be used in the commercial roofing to be manufactured.

According to this invention, the special fire-resistant bituminous coating composition can be formulated so that the flow resistance coefficient will be as high as 100. However, greatly improved fire resistance is obtained according to the invention when the flow resistance coefficient of the filler in the coating of the roofing in question is 75 or greater, although it is preferable to formulate the bituminous coating compositions so that the flow resistance coefficient of the filler in the bituminous coating composition is 90 or above.

As aforesaid, the different screen gradings of a fibrous mineral filler such as asbestos dust have been found by us to differ considerably in their effectiveness in imparting flow resistance to a bituminous coating composition. In view of these differences in effectiveness of the different screen gradings of a mineral fiber such as asbestos dust, we have, in order to indicate more definitely the amount of mineral fiber of given screen gradings that is required to effect stabilization of a bituminous composition, assigned to the different screen gradings what we have called the "screen factor" for each of the different gradings. Thus if the screen grading (-28+35) is taken as having a screen factor of unity, any screen grading that requires half the amount as compared with the screen grading (-28+35) will be twice as effective and will have a screen factor of 2. On the other hand, a screen grading that requires twice the amount as compared with the screen grading (-28+35) will only have half

the effectiveness and will have a screen grading of 0.5. In like manner, screen factors can be assigned to each of the other screen gradings.

The above-described test for measuring the flow resistance coefficient of a filler in a bituminous composition affords a convenient basis for setting up the screen factors of fibrous mineral fillers on a definite scale and, when the screen factor of a given screen fraction of a fibrous mineral is referred to herein, the screen factor as determined in the following manner is intended. The test for determining the flow resistance coefficient is carried out using the test apparatus and procedure above described except that in all cases the total filler is 55% by weight of the bituminous composition. The asphalt in all cases is oxidized straight run asphalt having a softening point of about 205° F. Slate flour about 85% by weight of which passes a 200 mesh testing sieve is used in all cases as the standard diluent filler, and the amount by weight of the particular screen grading of fibrous mineral to achieve a flow resistance coefficient of about 75, as ascertained by the average of a plurality of runs, is determined. Each sample is prepared using the asphalt saturated organic fiber felt above specified, namely, conventional organic fiber roofing felt weighing about 30 pounds per 100 square feet that has been saturated to the extent of about 175% by weight with asphalt having a softening point of about 150° F. As a standard, chrysotile asbestos dust of the grading (-28+35) is taken as having a screen factor of unity and the factor for each of the other gradings is calculated to this standard. By way of concrete example, it being the case that substantially 15% by weight of the bituminous composition of chrysotile asbestos dust having the screen grading (-28+35) (the total filler being 55% as aforesaid), is required to afford a flow resistance coefficient of substantially 75, and it also being the case that only about 3% by weight of the bituminous composition of chrysotile asbestos of the screen grading (-6+8) (the total filler again being 55%), also affords a flow resistance coefficient of about 75, the screen factor of chrysotile asbestos dust having the screen grading (-6+8) is seen to be about 5.

By way of further illustration, the "screen factors" of the different screen gradings of a typical chrysotile asbestos dust on the basis above mentioned are as follows:

| Screen Grading | Screen Factor |
|----------------|---------------|
| -6+8           | 5.0           |
| -8+10          | 3.8           |
| -10+14         | 2.5           |
| -14+20         | 1.9           |
| -20+28         | 1.4           |
| -28+35         | 1.0           |
| -35+48         | .8            |
| -48+65         | .7            |
| -65+100        | .5            |
| -100+150       | .4            |
| -150+200       | .3            |
| -200           | .2            |

It may be noted that in the case of the screen grading (-200), a flow resistance coefficient of 75 was not attained even when the total filler (55% by weight) consisted of this particular grading of asbestos dust. However, since this particular screen grading (-200) is nevertheless effective when combined with the more effective screen gradings, a screen factor of .2 has been assigned to this particular screen grading. Similarly, in

the case of any other fibrous minerals, a screen grading which, when employed to the extent of 55% by weight, does not attain a flow resistance coefficient of .75 is to be regarded as having a screen factor of .2.

The foregoing is seen to afford a convenient way of knowing and defining the flow resistance effectiveness of a fibrous mineral filler. Given the percentage by weight of each of the screen gradings of mineral fiber contained in a bituminous composition, the percentage by weight of each multiplied by the screen factor for each gives what we term herein and in the claims the "grading index" for each of the screen gradings; and, by adding the grading indices for the several screen gradings together, the grading index for the total mineral fiber is readily determined. By way of illustration, the grading index of the mineral fiber component of the above-mentioned typical embodiment of this invention is as follows:

| Screen Grading                        | Percent by Weight of Bituminous Composition | Screen Factor | Grading Index |
|---------------------------------------|---------------------------------------------|---------------|---------------|
| -6+8                                  | .1                                          | X             | .5            |
| -8+10                                 | .2                                          | X             | .8            |
| -10+14                                | .3                                          | X             | .6            |
| -14+20                                | .3                                          | X             | .6            |
| -20+28                                | .4                                          | X             | .6            |
| -28+35                                | 1.5                                         | X             | 1.5           |
| -35+48                                | 3.0                                         | X             | 2.4           |
| -48+65                                | 2.5                                         | X             | 1.8           |
| -65+100                               | 2.5                                         | X             | 1.2           |
| -100+150                              | 2.5                                         | X             | 1.0           |
| -150+200                              | 2.0                                         | X             | .6            |
| -200                                  | 5.7                                         | X             | 1.1           |
| Total grading index for mineral fiber |                                             |               | 12.9          |

It is apparent that in the formulation of a bituminous coating composition one can, from the screen analysis of a mineral fiber such as asbestos dust, determine the grading index of the mineral fiber employed and thereby determine the effectiveness of the mineral fiber in the amount used in stabilizing the bitumen in the coating composition. As mentioned above, we have found that in highly mineralized coatings one can, by attaining the critical point at which there is a sudden increase in the flow resistance coefficient, provide a fire-resistant roofing even though fibrous mineral is not employed. However, the coating composition is improved when mineral fiber is present in an amount and of such screen gradings that the ratio of the grading index to the per cent. by weight of bitumen in the composition is at least 1 to 8 and it is preferable that the ratio be about 1 to 6. These ratios are applicable for the range from 20% to 45% by weight of bitumen in the composition and are especially suitable when the bitumen is of the range 20% to 35% by weight. When the bitumen content of the bituminous composition is of the range 35% to 45% by weight, it is usually desirable that the ratio of the grading index to the per cent. by weight of bitumen be about 1 to 6 and preferably about 1 to 3. Referring to the foregoing example, the grading index of the fibrous mineral was seen to be 12.9, and since the per cent. by weight of asphalt in the composition is 32% by weight, the ratio of the grading index to the per cent. by weight of asphalt is about 1 to 2.5, which is well within the minimum ratios just mentioned.

When reference is made herein to "screen factor" and "grading index" of fibrous mineral filler, the reference is made to these values when determined as hereinabove described. When, however, reference is made to flow resistance coefficient

of a filler or filler mixture, the flow resistance coefficient, unless otherwise specified, is that of the filler or filler mixture in whatever amount it is present as commingled with the kind of asphalt employed in the bituminous composition, the bituminous composition being tested as applied to the base sheet of the commercial product.

In determining the screen fractions or gradings of fibrous or other mineral fillers that are referred to herein, 8 inch diameter testing sieves of the W. S. Tyler Company sieve series, meeting A. S. T. M. Standard E11-39 for Sieves for Testing Purposes have been used. A quantity of filler to be screened, ranging from 200 to 300 grams, is placed in the uppermost of a series of testing sieves and subjected to suitable agitation as in a standard W. S. Tyler Company Ro Tap sieve shaking machine for a period of five minutes in order to separate the original filler roughly into fractions retained in the different testing sieves. This operation is repeated, if necessary, in order to obtain about 100 to 200 grams of the desired screen fraction, which fraction is then individually rescreened for 15 minutes, using the Ro Tap sieve shaking machine or the equivalent in order to remove any fines contained therein. The resulting screen fraction is the material that has passed the coarser screen and is retained on the finer screen.

As aforesaid, it is essential that the high flow resistance coefficient be attained in a bituminous composition that does not exceed a predetermined plasticity value at 400° F. The fire-resistant bituminous compositions of this invention fall within the narrow range wherein the flow resistance coefficient exceeds the minimum above mentioned, but have a plasticity value at 400° that does not exceed 1500 grams and that preferably does not exceed 1000 grams. The plasticity value at 400° F. of the bituminous composition described in the exemplary embodiment of this invention is about 1125 grams.

The plasticity value of the bituminous composition has been determined by us, using a Wagner-Bowen mixing bowl plasticimeter, manufactured by E. E. W. Bowen, Bethesda, Maryland. For testing bituminous compositions of the character mentioned herein, we have made certain modifications in this test apparatus. In view of this fact and further in view of the fact that we do not know of any available publication wherein this type of apparatus is described in detail, we have shown in the drawings, Fig. 18 to Fig. 23C, the testing apparatus which we have employed and a description of the apparatus and its operation follows. When reference is made herein or in the claims to Wagner-Bowen plasticity value, the plasticity value as determined by this test is intended.

The Wagner-Bowen plasticimeter consists of a suitable base 100 which comprises in housing 143 suitable gear means (not shown) for rotating the vertical shaft 101 by power supplied from the motor 102. The shaft 101 carries for rotation at the upper end thereof the horizontally-disposed disk-shaped support 103 to the top of which is secured the bowl 104 by means of screws 105. By this arrangement, the bowl 104 can be rotated by operation of the motor 102, and any suitable means can be provided for maintaining the rotation of the bowl at a predetermined constant speed.

Emanating from the base 100 are arms 106 and 106' which carry on the upper ends thereof the cross bar 107. At the upper end of each arm 106

and 106' is a yoke 108 which is pivoted to lug 109 and which is provided with a thumb screw 110 in threaded engagement therewith so that, by loosening the thumb screw 110, the yoke 108 can be swung outwardly, permitting removal of the cross bar 107. At each end of the cross bar 107 is a positioning pin 111 by which the position of the cross bar is determined.

The cross bar 107 carries the means determining the plasticity of material in the bowl 104. Carried at the lower end of shaft 112 is the mixing blade 113, the vertical position of which relative to the bowl 104 is adjustable by nuts 114 which secure the shaft 112 to the cross bar 107. Adjacent the end of the mixing blade 113 is the thermometer 115 carried in a guard 116 attached to bracket 117 which in turn is secured at the upper end to the cross bar 107. Carried by the lower end of the shaft 118 is the smoothing blade 119. The shaft 118 and smoothing blade 119 are urged downwardly by the expansion spring 120 between the annular washer 122 and the sleeve 121 in which the shaft 118 is vertically slidable. The vertical position of the smoothing blade 119 is determined by the thumb screw 123 which rests against the upper end of sleeve 121 and which is in threaded engagement with the upper end of the shaft 118. Also rigidly secured to the cross bar 107 is the rod 124, the lower end of which can be adjusted so as to be a predetermined distance from the bottom of the bowl 104 by nuts 125.

At the center of the cross bar 107 is the bearing 126 for the vertical shaft 127 that is mounted for rotation therein at a given vertical position. Rigidly secured to the shaft 127 by means of the collar 128 is the arm 129 which carries the small cylindrical drag tool 130 at the lower end thereof. Carried by the upper end of shaft 127 and rotatable therewith is the arm 131, the outer end of which has a small amount of play for angular movement with the shaft 127 between opposed adjustable stop screws 132.

A horizontally-disposed stub shaft 133 is fixedly carried by arm 106' and pivotally mounted thereon is the T-shaped scale beam member comprising the vertically-extending arm 134 and the arms 135 and 136 extending horizontally on opposite sides of the stub shaft 133. Pivotally secured at the end of the arm 135 is the weight pan 137 and pivotally secured at the end of arm 136 is the counterweight 138 which substantially counterbalances the weight pan about stub shaft 133. Between the end of arm 131 and the end of arm 134 is the tie rod 139. One end of the tie rod 139 has a turned-down portion 140 which slips through an opening of corresponding size in the end of arm 131 to provide pivotal movement with respect thereto. The other end of tie rod 139 is in threaded engagement with a yoke member 141 which is pivotally mounted with respect to the upper end of arm 134. If desired, a fixed stop arm 144 can be provided for convenience in restraining movement of arm 134 when the tie rod 139 is disengaged from arm 131. The contents of the bowl 104 can be heated as by the gas burners 142.

In the operation of the plasticimeter, the bowl 104 is rotated in a clockwise direction, and, as the bowl continues to operate, the mixing blade 113 scrapes the heated contents of the bowl away from the outside bottom portion thereof and the thermometer 115 records the temperature of the contents of the bowl at this point. The contents of the mixing bowl are next carried under the smoothing blade 119 which smooths the con-

tents of the bowl to a predetermined level above the outer portion of the bottom of the bowl. The lower end of the rod 124 serves as a check to determine whether the smoothing blade 119 is smoothing the contents of the mixing bowl to the desired level, and, if it is not, the vertical position of the smoothing blade 119 is adjusted by thumb screw 123. The heated contents of the bowl at the predetermined desired level therein are then carried past the drag tool 130 and this tends to rotate the shaft 127 in a clockwise direction and to pull the weight pan 137 upwardly through the system of lever arms and tie rod hereinabove described. The greater the plasticity (i. e., the heavier the consistency) of the contents of the bowl 104, the greater will be the drag on the drag tool 130 that tends to elevate the weight pan 137. By placing weights on the weight pan 137 and while continuing to rotate the bowl 104, the device can be brought into a state of equilibrium so that the end of the arm 131 will be approximately midway between stop screws 132—132, and the weight in grams required to achieve this condition of equilibrium for a particular composition contained in the mixing bowl is the Wagner-Bowen plasticity value. This value is dependent upon the dimensions of the apparatus and the manner of use of the apparatus in making the determination. The essential dimensions of the apparatus shown in the drawings are:

|                                |                                |
|--------------------------------|--------------------------------|
| a, 3 $\frac{1}{8}$ inches      | r, 4 $\frac{1}{8}$ inches      |
| b, 9 $\frac{5}{8}$ inches      | s, 1 $\frac{1}{4}$ inches      |
| c, $\frac{1}{8}$ inch          | t, 2 $\frac{1}{2}$ inches      |
| d, 8° angle                    | u, 2 $\frac{5}{8}$ inches      |
| e, 7 $\frac{1}{8}$ inches      | v, 1 $\frac{1}{8}$ inches      |
| f, 4° angle                    | w, 9° angle                    |
| g, 3 $\frac{5}{8}$ inches      | x, 5 $\frac{1}{8}$ inch radius |
| h, 2 $\frac{3}{8}$ inches      | y, 11° angle                   |
| i, 2 $\frac{7}{8}$ inches      | z, 1 inch                      |
| j, 2 $\frac{1}{4}$ inches      | aa, 3 $\frac{1}{8}$ inches     |
| k, 4 $\frac{3}{4}$ inch radius | bb, 2 $\frac{3}{4}$ inches     |
| l, 1 $\frac{1}{8}$ inch radius | cc, $\frac{3}{4}$ inch         |
| m, $\frac{1}{8}$ inch          | dd, $\frac{5}{8}$ inch         |
| n, 2 $\frac{1}{8}$ inches      | ee, $\frac{1}{4}$ inch         |
| o, 1 $\frac{1}{8}$ inches      | ff, 24° 15' angle              |
| p, 2 $\frac{1}{8}$ inches      | gg, $\frac{5}{8}$ inch radius  |
| q, 2 $\frac{1}{8}$ inches      | hh, $\frac{1}{8}$ inch         |

The dimensions of the mixing blade 113 and of the smoothing blade 119 are indicated on the face of the drawings.

The Wagner-Bowen plasticity values at 400° F. given herein are determined in the following way. The height of the lower end of the measuring rod 124 from the bottom of the bowl 104 is adjusted so as to be  $\frac{7}{8}$  inch. The height of the bottom of the drag tool 130 from the bottom of the bowl is set so as to be  $\frac{1}{4}$  inch. The weight of the composition to be tested is approximately 1500 grams. The weight is not critical provided the thickness of the composition as it leaves the smoothing blade just clears the lower end of the measuring rod 124. The composition is mixed while in the bowl 104. Throughout the test the bowl 104 is rotated at the rate of 60 rotations per minute. The bitumen that is used in the composition while in a heat-liquefied condition is poured into the bowl while the bowl is rotating. The bitumen is brought to a temperature of 400° F. by the burners and, while maintaining the temperature of 400° F., the filler material is added in small increments until it has all been incorporated. The smoothing blade 119 is then adjusted so that the composition as it leaves the smoothing blade just clears the lower

end of the measuring rod 124. Weights are then placed on the weight pan 137 until the arm 131 is brought to a position between the stop screws 132, the weight to bring about this condition of equilibrium being recorded. Such recordings are made every five minutes until the recorded weight becomes constant for three consecutive readings. The weight in grams for the last three consecutive readings is taken as the Wagner-Bowen plasticity value of the composition at 400° F.

As mentioned above, it is not essential that a mineral fiber filler such as asbestos dust be included in the bituminous composition. Thus the asbestos dust may be omitted and the filler may consist only of limestone dust or slate flour. In such case, however, a greater percentage of filler to bitumen is required, the critical value for powdered limestone dust usually being in the neighborhood of 75 to 80% by weight of limestone dust in the composition. Other filler material may also be used, but the critical amount differs in the case of each filler. In the case of each filler, the effect of attaining and exceeding a critical value has been noted by us for, upon the addition of any filler material, there is comparatively little effect on flow resistance coefficient up to the critical point, followed by a sudden and very great increase in flow resistance coefficient as soon as the critical point is reached. Thus, for slate flour 85% by weight (-200) when used by itself, the critical point is usually around 65% by weight of the coating composition. In the case of silica flour 85% by weight (-200) the critical point is in the neighborhood of 70% by weight of the composition. Kaolinitic type clays are also suitable. Thus for one type of kaolinitic type clay which is known commercially as "Girard" clay (produced by United Clay Mines Corp., Trenton, New Jersey), the critical value is usually around 60% by weight of the composition, while for another type of kaolinitic type clay which is sold under the name "Tako" (produced by Thomas Alabama Kaolin Co.), the critical point is usually somewhat higher, that is, around 65% by weight of the composition. For one variety of talc, the critical value is about 70% by weight of the composition. In connection with the foregoing, it may be pointed out that the figures above given as to critical percentages are subject to slight variation due to the fact that the critical percentage for a given filler will vary somewhat, depending upon the manner of grinding the filler to a pulverulent condition, the character of the bitumen with which it is mixed, and the thoroughness of the mixing. However, from the foregoing, it is apparent that there is a critical point at which for a given filler-bitumen composition there is the sudden and very great increase in flow resistance coefficient. There are a number of other filler materials that may likewise be employed, such as precipitated calcium silicate hydrate, hydrated Portland cement, lime plaster, fly ash and the like. Also filler mixtures of various kinds may be employed. The upper limit as to the amount of such filler material that may be incorporated is determined by the Wagner-Bowen plasticity value at 400° F. as measured by the plasticity test above mentioned. Usually, the range of permitted filler content is confined within limits of a few per cent. by weight of the filler that is contained in the composition, and in the case of some filler materials the permitted maximum plasticity value for worka-

bility is exceeded before the critical flow resistance coefficient is attained, and, if a particular filler is of this character, then such filler material may not satisfactorily be employed. However, in the case of those fillers which, within the permitted limit of plasticity value, may be added to obtain the high flow resistance coefficient above mentioned, any filler in the form of finely-divided solid water-insoluble heat-resistant mineral filler may be employed. By "heat-resistant" any material is intended which is sufficiently heat-resistant so that it will retain structural integrity when subjected to flame temperature while incorporated in the roofing. In this connection, substances such as chrysotile asbestos, Canadian picrolite, hydrated Portland cement, etc., are regarded as heat-resistant even though they contain water of constitution which may be driven off at temperatures at or below flame temperatures. In connection with the foregoing, it may be pointed out that the Wagner-Bowen plasticity value and the flow resistance coefficient are different properties that are not affected proportionally by increasing the amount of filler in a bituminous composition.

As mentioned above, it is desirable to include in the bituminous composition as at least part of the filler material a finely-divided mineral fiber such as asbestos, the particles of which are such as to pass a 6 mesh standard testing sieve and be retained on a 200 mesh standard testing sieve. Also as aforesaid, such fibrous minerals include fractions that, when used by themselves and in amounts less than 55% by weight of the composition, afford a flow-resistance coefficient of 75 or greater. The preferred mineral fiber filler is chrysotile asbestos dust or shorts. Other asbestosiform mineral fibers that may be used are Canadian picrolite, amosite, anthophyllite, tremolite and actinolite. Other mineral fibers of the particle size mentioned may likewise be employed, such as mineral wool and glass fibers. The term "mineral wool" includes various fibrous products obtained by attenuating into fibrous form suitable fused materials such as rock or slag.

Another suitable fibrous material is a comminuted mixture of hydrated Portland cement and asbestos fiber, the hydrated Portland cement having become set with the asbestos fiber distributed therethrough. A convenient source of such material is asbestos-cement roofing scrap. Asbestos-cement roofing scrap usually contains about 20% to 35% by weight of asbestos fiber and about 65% to 80% by weight of hydrated Portland cement. Heretofore such scrap has been regarded as unavoidable waste of no commercial value. However, by subjecting the scrap to a disintegrator, such as a hammer mill, until the particle size is of the order of that mentioned in connection with asbestos fibers, the resulting mass contains a multiplicity of the short asbestos fibers to which the hydrated Portland cement adheres as nodules, and for this reason this material is essentially a fibrous material and is to be regarded as a finely-divided fibrous mineral filler.

Another material which is somewhat similar to asbestos-cement in that the material contains mineral fibers together with non-fibrous material is disintegrated fiber-bearing serpentine rock. Since disintegrated fiber-bearing serpentine rock contains fibrous particles, such disintegrated serpentine rock is regarded as one form of fibrous mineral which is suitable for use in practicing this invention. However, depending upon the physical structure and fibrous mineral

content of the particular serpentine rock that is used, the proportion of fiber contained therein is subject to some variation, but, as pointed out below, this merely has the effect of varying somewhat the screen factors of the various screen gradings of the disintegrated serpentine rock as calculated to chrysotile asbestos dust of the screen grading ( $-28+35$ ) which has a screen factor of unity. Moreover, disintegrated serpentine rock is of such character, that in order to liberate the fibrous material contained therein it should pass a 20 mesh testing sieve, and, when reference is made herein to disintegrated fiber-bearing serpentine rock, only that serpentine rock which has been disintegrated so that it passes a 20 mesh testing sieve is intended, since the individual particles of such coarser gradings are not fibrous in character but granular (are not fibrous mineral as this term is used herein) and since such coarser gradings are ineffective in producing highly fire-resistant roofings.

With regard to the fibrous mineral materials other than asbestos-form mineral fibers, it is not necessarily the case that a particular screen grade of, for example, asbestos-cement or mineral wool, will have the same screen factor as that of chrysotile asbestos fiber. In fact, even as between different types of asbestos-form mineral fiber, there are some variations in this regard. However, utilizing chrysotile asbestos fiber as the standard, chrysotile asbestos fiber of the screen grading ( $-28+35$ ) having a value of unity, the screen factor of the screen gradings of the different fibrous minerals is determinable in the same way that the screen factor of each of the various screen gradings of chrysotile asbestos fiber is determinable as has been described hereinabove. For example, the screen factor of asbestos cement prepared from asbestos-cement roofing scrap and of the screen grading ( $-28+35$ ) will be about 3 as compared with the screen factor of unity for chrysotile asbestos fiber of the same screen grading. The screen factor of mixtures of fibrous minerals will bear a similar relationship to the screen factor of unity of chrysotile asbestos of the screen grading ( $-28+35$ ). When a mixture of fibrous minerals is employed, it is preferable that all or at least a major proportion of the fibrous mineral be selected from asbestos-form mineral fibers, disintegrated asbestos-cement, and disintegrated fiber-bearing serpentine rock.

Of the filler materials above mentioned, chrysotile asbestos fiber and Canadian picrolite usually contain about 12% to 15% of water of constitution liberatable at temperatures approaching flame temperatures. The other asbestos-form mineral fibers are low in water of constitution. Some of the non-fibrous filler materials likewise contain water of constitution that is liberatable at or adjacent flame temperatures. Thus kaolinitic type clays, powdered serpentine rock, calcium silicate hydrate and hydrated Portland cement contain 10% to 13% or more of water of constitution that is liberatable at or below flame temperatures, although impure clay may contain as low as 5% of water of constitution. When the filler material contains water of constitution liberatable at or below flame temperature, the liberation of moisture causes the bituminous composition to develop pores to a greater extent than otherwise when the bituminous composition is exposed to flame temperatures and this is desirable since the pores tend to augment the heat insulating efficiency of the mat-like residue that

is formed upon exposure of the bituminous coating composition to flame temperature. It is desirable that the bituminous coating composition have incorporated therein a filler material containing water of constitution which water of constitution liberatable at or below flame temperature amounts to at least about 5% by weight of the coating composition.

In the selection of filler material for use in the highly fire-resistant bituminous composition of roofings embodying this invention, the materials such as powdered limestone, slate flour, talc, silica flour, kaolinitic clays, and the like, may be employed in the state of subdivision in which they ordinarily occur on the market. The bulk of such materials will pass a 200 mesh testing sieve, and it is preferable that at least 90% by weight of the non-fibrous mineral filler material pass a 100 mesh testing sieve. It is ordinarily desirable that the coating composition contain less than about 10% by weight of the total filler in the bituminous composition of granular particles of non-fibrous filler that are retained on a 14 mesh testing sieve. Referring to the filler as a whole, including possible presence of mineral fiber filler, it is desirable that at least half by weight of the mineral filler pass a 100 mesh testing sieve, and preferably at least  $\frac{2}{3}$  by weight of the total filler material should pass a 100 mesh testing sieve. As aforesaid, the critical point at which the great increase in flow resistance value is attained will vary depending somewhat upon the state of subdivision of the filler material, but it is not regarded as necessary herein to prescribe exact limits as to particle size, since proper particle size is inherent provided the filler in question, when incorporated with the bitumen of the bituminous composition, has a flow resistance coefficient above the minimum hereinabove given and provided the composition has a Wagner-Bowen plasticity value not above the maximum hereinabove given. The Wagner-Bowen maximum plasticity limit also precludes the employment in the composition of an excessive amount of fibrous mineral material of the coarser screen gradings, since the presence of fiber of substantial length greatly increases the Wagner-Bowen plasticity value. It may be mentioned, however, that such mineral fibers that come up within the grade of asbestos known as "fiber" according to the classification of the Quebec Asbestos Producers Association and which are the type in general commercial use are undesirable for use in bituminous coating compositions according to this invention. Thus such fibers tend to become entangled in clumps or clots which result in non-uniform distribution so that the coating is too irregular to be commercially acceptable, the fire resistance is impaired due to poor adhesion to the base sheet and zones of inadequate protection, the weather resistance is impaired due to zones of inadequate coverage of the base sheet and the like. It is of great practical importance that the fire-resistant coating compositions of this invention are spreadable, that is, can be readily prepared and applied with the production of a good waterproof coating of uniform thickness and consistency and of long weathering life using ordinary roofing machines. The above-mentioned limits as to Wagner-Bowen plasticity value of the bituminous coating compositions of this invention insure good spreadability. It is ordinarily desirable, for reasons above mentioned, that the ratio of the grading index of the fibrous mineral to the percent by weight of bitumen in the composition be not

greater than about 1 to 7 and preferably not greater than about 1 to 1.

With regard to the bitumen that is employed in the special fire-resistant bituminous composition, it is usually preferable to employ an asphalt having a softening point of about 180° F. to about 220° F. Somewhat more generally, the asphalt should have a softening point above 160° F. and usually the softening point of the bitumen should be below about 275° F., if the plasticity value at 400° F. is to be kept below the maximum mentioned hereinabove. The softening points referred to herein are determined by the standard ring and ball softening point test. The amount of bitumen, depending upon the critical point for the filler that is used, will be between about 20% and 45% by weight of the bituminous composition (the amount of filler running from 55% to about 80% by weight of the bituminous composition). In addition to asphalts derived from Mid-Continent crudes, asphalts from Mexican, Venezuelan and Colombian crudes are also suitable. Moreover, other bitumens such as pitches, coal tar and the like may also be used in the practice of this invention. While it has been mentioned that the flow resistance coefficient of a filler is usually somewhat higher in the case of cracked asphalts as compared with other asphaltic materials, cracked asphalts do not have as long weathering life, and for this reason it is usually preferable to use the usual type of roofing asphalt for direct exposure to sun and weather.

In the foregoing example of the practice of the invention, the special bituminous coating material was applied at the rate of 45 pounds per 100 square feet of the roofing. It is usually desirable to apply the special coating composition to the weather side of the base sheet so that the coating layer will weigh about 20 to about 60 pounds per 100 square feet, although about 30 to 50 pounds per 100 square feet is usually preferable. In the foregoing example wherein the special bituminous coating contained substantially 68% of filler and the coating was applied at the rate of 45 pounds per 100 square feet, the amount of filler in the coating composition constituted about 30 pounds per 100 square feet of the roofing material. For prepared roofing materials, it is usually desirable that the roofing material contain in one or more layers such as a surface layer or a backing or other layer, sufficient of the special bituminous coating composition so that the roofing material will contain at least 15 and preferably 22 pounds per 100 square feet of the filler material. By varying the number and thickness of the layers of special bituminous coating composition in a prepared roofing material or in a roof covering, varying degrees of fire-retardant effectiveness can be attained. The special bituminous composition of this invention is especially effective when it is disposed in a roofing so as to occur in a plurality of layers separated by felt or other sheet material, for example, as shown in Figs. 3 and 4 or as shown in Figs. 7 and 8. In such plural layer construction, it is preferable that each of at least two of the layers of special bituminous composition contain at least about 11 pounds per 100 square feet and preferably 20 pounds per 100 square feet of the heat-resistant filler material, and that the roof covering as a whole contain at least 22 pounds per 100 square feet and preferably 40 pounds per 100 square feet of the heat-resistant filler material.

Roofings comprising a plurality of layers of the

75

special bituminous coating composition need not necessarily be assembled on the job but may be preformed at the factory. Such a multilayer roofing is illustrated in Fig. 10. This roofing material contains three layers of asphalt impregnated felt. Between the layers of felt are layers 81 of the special bituminous coating composition. In addition, there is a surface layer 82 of the special bituminous coating composition. The felt layers 80 may, if desired, be composed of asbestos fiber; but, instead of asbestos fiber felt, ordinary organic fiber felt may be used, since the special coating composition of this invention in itself affords high fire resistance. The top layer 82 may, if desired, be omitted.

While felt sheet material has been mentioned hereinabove as the strain-resisting element of roofing and roofing structures embodying this invention, it is apparent that any other suitable sheet material either fibrous or non-fibrous, either foraminous or non-foraminous, adapted to afford desired strength characteristics may be employed. Thus fabrics other than felt may be employed, such as woven fabrics or fabrics of unspun bonded fibers. The base sheet may, if desired, be saturated with a waterproofing material or may be dry. Sheet material such as composition board or insulation material may be employed. Plain or corrugated or indented sheet metal may also be used as the base sheet. Ordinary roofing felt made of organic fibers is, however, the most inexpensive sheet material, and notwithstanding the combustibility of such sheet material, roofing comprising it can, according to this invention, be made highly fire-resistant. If desired, non-combustible fibers can be incorporated in the felt or other fibrous base sheet to augment the fire resistance of the roofing.

It is one of the advantages of this invention that the new roofing herein defined possesses high fire resistance without sacrifice of other properties required for a roofing and without substantial increase in cost compared with conventional roofings heretofore manufactured. The new roofing of this invention has very good weathering characteristics and is tough and pliable. Thus a typical preformed roofing material such as a shingle can be bent 180° in two seconds around a 4 centimeter mandrel with the fire-resistant special coating composition on the outside without cracking the coating through to the felt base, the test being made at 77° F. It is desirable that a roofing having a bituminous waterproofing coating be sufficiently pliable to be bent 180° in two seconds about a mandrel 10 centimeters in diameter at 77° F. with the coating on the outside without cracking the coating through to the base on which it is applied, and any such coating or layer is referred to herein as "pliable" at ordinary temperatures.

In our aforesaid application Serial No. 399,024, we have disclosed that the problem of the blistering of roofings can be met by effecting a great increase in the viscosity and strength of the bituminous coating composition and have claimed such highly blister-resistant roofings wherein the bituminous coating layer contains at least 45% by weight of bitumen. The highly mineralized coatings of the present invention, which contain less than 45% by weight of bitumen, can be made with the high viscosity and strength characteristics requisite for minimizing blistering but, in order to do so, the softening point of the bitumen should be above 200° F. For purposes of brevity, reference is made

herein to the specification of our said application, Ser. No. 399,024 as though the same were set forth herein. Those properties given in our aforesaid application as definitive of highly blister-resistant bituminous coatings are that the bituminous coating composition have a softening point above 300° F., have a viscosity at 170° F. greater than  $4 \times 10^7$  poises, and have a tensile strength at 170° F. of at least 150 gm. per sq. cm. For a suitable roofing, the coating composition also should have a work capacitance at 77° F. of at least 2000 gm. cm. per cu. cm. and a per cent. elongation at 77° F. of at least 35. The filler should have a preferential affinity for the bitumen in the composition as against water at 185° F. Preferably, the viscosity at 170° F. of the highly blister-resistant bituminous composition is at least  $20 \times 10^7$  poises. The measurement and significance of these properties is fully explained in our aforesaid application Ser. No. 399,024. The bituminous coating layer should, in order to provide high blister resistance, be applied at the rate of at least about 20 pounds per 100 square feet.

While this invention has been described in connection with certain illustrative embodiments thereof, it is to be understood that this has been done for the purpose of exemplification. Accordingly, the scope of this invention is to be governed by the language of the following claims construed in the light of the foregoing description of our invention.

We claim:

1. A roofing having high fire resistance and high blister resistance comprising sheet-like base material and carried by said sheet-like base material a waterproofing layer of thermoplastic bituminous composition, said bituminous composition containing bitumen having a softening point above 200° F. and not above 275° F. and of the range between 20% and 45% by weight of said bituminous composition, said bituminous composition containing intimately commingled and distributed uniformly throughout finely-divided solid water-insoluble heat-resistant mineral filler of the range above 55% to 80% by weight of said composition which has a preferential affinity for said bitumen as against water at 185° F., said bituminous composition having a Wagner-Bowen plasticity value at 400° F. not greater than 1500 grams, having a softening point above 300° F., having a viscosity at 170° F. greater than  $4 \times 10^7$  poises, having a tensile strength at 170° F. of at least 150 gm. per sq. cm., having a per cent. elongation at 77° F. of at least 35, and having a work capacitance at 77° F. of at least 2000 gm. cm. per cu. cm., the said filler contained in said bituminous composition having a flow resistance coefficient of at least 75 when said composition carried by said sheet-like base material is exposed to flame temperature under the flow resistance test as defined herein, and said bituminous composition providing a pliable weather-resistant layer of the hot-spread coating type which is integrally bonded with said sheet-like base material and

is of a thickness throughout not less than corresponding to about 20 pounds per 100 square feet throughout the extent of said layer where said layer is designed to provide blister resistance.

2. A roofing material having high resistance to fire and high blister resistance comprising a sheet-like base material and carried by said sheet-like base material a waterproofing layer of thermoplastic bituminous composition, said bituminous composition containing bitumen having a softening point above 200° F. and not above 275° F. and of the range between 20% and 45% by weight of said composition, and said bituminous composition containing intimately commingled and distributed uniformly throughout finely-divided solid water-insoluble heat-resistant mineral filler of the range above 55% to 80% by weight of said composition which has a preferential affinity for said bitumen as against water at 185° F., said bituminous composition having a Wagner-Bowen plasticity value at 400° F. which is substantially greater than 250 grams and which is not greater than 1500 grams, having a softening point above 300° F., having a viscosity at 170° F. of at least  $20 \times 10^7$  poises, having a tensile strength at 170° F. of at least 150 gm. per sq. cm., and having a work capacitance at 77° F. of at least 2000 gm. cm. per cu. cm., the said filler contained in said bituminous composition having a flow resistance coefficient of at least 75 when said composition carried by said sheet-like base material is exposed to flame temperature under the flow resistance test defined herein, and said layer being of the hot-spread coating type integrally bonded with said sheet-like base material and being applied to said sheet-like base material at a rate such that the thickness corresponds to about 20 pounds to about 60 pounds per 100 square feet of said roofing material and said roofing material being pliable at 77° F.

HAROLD W. GREIDER.  
GEORGE ARTHUR FASOLD.

#### REFERENCES CITED

The following references are of record in the file of this patent:

| UNITED STATES PATENTS |                |               |
|-----------------------|----------------|---------------|
| Number                | Name           | Date          |
| 732,663               | Stempel        | June 30, 1903 |
| 1,751,690             | Faber          | Mar. 25, 1930 |
| 1,949,229             | Yeager         | Feb. 27, 1934 |
| 2,157,696             | Greider et al. | May 9, 1939   |
| 2,158,772             | Beckwith       | May 16, 1939  |
| 2,178,770             | Zaisser        | Nov. 7, 1939  |
| 2,317,209             | McCluer        | Apr. 20, 1943 |
| 2,326,723             | Fasold et al.  | Aug. 10, 1943 |
| 2,354,593             | Greider et al. | July 25, 1944 |
| 2,424,234             | Greider et al. | July 22, 1947 |

#### OTHER REFERENCES

Petroleum Zietschrift, Vol. XXIX, Nr. 45 (1933), pp. 1-12.